

Patented Aug. 1, 1950

2,517,044

1. A process for making power transmission fluids comprising the steps of adding to a mixture of castor oil and glycerine a quantity of alkali hydroxide or alkoholate, the quantity being such that the free acidity of the castor oil is neutralised, and then adding to the mixture a quantity of glycerol monoether, the quantity being such that the final product has a viscosity of approximately 1000 centistokes at 40° C.

# UNITED STATES PATENT OFFICE

2,517,044

## PROCESS FOR MAKING POWER TRANSMISSION FLUIDS

William Percival Smith, Leamington Spa, England, assignor to Automotive Products Company Limited, Leamington Spa, England

No Drawing. Application September 5, 1944, Serial No. 552,820. In Great Britain July 26, 1943.

6 Claims. (Cl. 252—76)

1. This invention relates to power transmission fluids of the type comprising castor oil and a diluent such as an ether or ester of glycol or glycerine.

Castor oil is a well known ingredient of power transmission fluids owing to its lubricating properties and the fact that it does not adversely affect the rubber parts of brake mechanism nor corrode the metal parts; and also the extended range of temperatures over which its viscosity has little variation, and mixtures of glycol ethers and castor oil have been popular for this purpose for a number of years.

A solution of castor oil in Cellosolve in the proportion of 35% castor oil, 65% Cellosolve which has been brought to practical neutrality by means of a solution of potash in Cellosolve, has been standardised and will remain liquid down to a temperature of  $-40^{\circ}\text{C}$ .

The exacting conditions of modern aircraft work make it necessary to produce power transmission fluids which will remain liquid at much lower temperatures and still retain the same properties as the castor oil-Cellosolve mixtures at the normal and elevated temperature ranges.

It has now been found that if the neutralisation step is carried out in such a way, when making a castor oil-Cellosolve mixture, that before adding the bulk of the Cellosolve a somewhat greater amount of caustic potash is added than that required to neutralise the free acidity of the castor oil, and at the slightly elevated temperatures normally employed in mixing these fluids, viz. about  $30^{\circ}\text{--}40^{\circ}\text{C}$ , if sufficient time is allowed to elapse (determined by alkalinity tests) to allow of a certain amount of saponification to take place until the neutral point is reached and thereupon the bulk of the Cellosolve is added, a solution may be produced which has a considerably increased water tolerance and will remain liquid at temperatures as low as minus  $60^{\circ}\text{C}$ .

The 35% : 65% castor oil-Cellosolve mixture is a standard mixture and has been found to meet most of the requirements of power transmission fluids, except the highly exacting low temperature conditions required for certain purposes, and the fact that these low temperature standards can now be attained without altering the composition of the fluid, is a discovery of the first importance and is believed to be of general application where neutralised castor oil-glycol monoether fluids are made up.

It was believed that the saponification products thus formed in the castor oil were an essential ingredient in the castor oil-diluent low temperature fluid.

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

Consequently, the alkali hydroxide or alkoholate is added with a quantity of glycerol monoether, the quantity being such that the final product has a viscosity of approximately 1000 centistokes at  $40^{\circ}\text{C}$ .

ricinoleate-glycol monoether fluid. Accordingly the invention includes a process for preparing a fluid for transmission of power which comprises adding sodium or potassium to a mixture of glyceryl tri-ricinoleate and a glycol monoether (e. g. a 35% : 65% mixture of glyceryl tri-ricinoleate and Cellosolve).

The invention includes the step of separating the saponification products from the tri-ricinoleate reaction products by washing with water until no more soap is removed whereby a modified ricinoleate oil is obtained which can be used for making a power transmission fluid by mixing with a glycol monoether e. g. with Cellosolve to bring the proportions to 35% oil and 65% Cellosolve.

The amount of alkali hydroxide or alcoholate which must be added to obtain optimum results varies according to the conditions obtaining during mixing, but this can easily be determined by a previous trial accompanied with a water tolerance test.

According to one way of carrying out the invention, castor oil and Cellosolve may be mixed in the proportion of 35% castor oil and 65% Cellosolve, but conveniently only a small proportion, say  $\frac{1}{3}$  of the Cellosolve is mixed with the castor oil in the first instance and the required amount of alkali, for example potash, may be mixed with this portion of the Cellosolve before it is mixed with the castor oil, and when the Cellosolve solution of the potash is mixed with the castor oil, the mixture may be allowed to stand until tests show that the solution has lost its alkaline reaction and become neutral.

In order that the interval required for completing this reaction is not too long, it is desirable to raise the temperature of the ingredients somewhat, the actual temperature chosen being arranged so that a convenient interval for making tests is allowed. This may be effected by storing the castor oil in a warm room, say at about 40°-45° C. As soon as neutrality is reached, the remainder of the Cellosolve is added so that no further reaction takes place owing to the dilution of the caustic potash.

The following examples give specific ways of carrying out the invention by way of illustration only:

#### Example 1

205 gallons of castor oil (which has been stored at a temperature of 45° C.) was pumped into a mixer and mixed with 122 gallons of Cellosolve in the following manner:

The castor oil contained in 5 drums was pumped into the mixer, one drum at a time, and in between each drum a similar proportion of the Cellosolve was pumped in, but before the last drum of Cellosolve was pumped into the mixer 4 gallons of filtered solution of potash in Cellosolve, containing 35 ozs. potash per gallon of Cellosolve, was placed into the last drum and roughly mixed, and then this drum was pumped on to the top of the contents in the mixer, it being arranged so that the Cellosolve containing the potash is pumped in on the top of the layer of Cellosolve, so that there is no appreciable contact of castor oil and potash solution until all is ready for the mixing. Mixing was then commenced until a homogeneous solution was obtained and a sample was drawn out for testing (the temperature being found to be 30° C.) and was found to have a water tolerance (measured by adding water to 100 cc. sample) of 19; and alkalinity test was made by titrating 20

ccs. of the fluid with N/10 HCl using phenol phthalein as indicator. This first test showed that 0.8 cc. of acid was required before neutrality was reached. After standing five minutes and agitating for 20 minutes, similar tests showed water tolerance 20 alkalinity 0.2 cc. The fluid was then allowed to stand without agitation for a further 20 minutes when it gave water tolerance 21 and alkalinity 0.01 cc. At this point a further 258 gallons of Cellosolve were pumped into the mixture and tests showed water tolerance 20.7, alkalinity faintly on the acid side of neutral, viscosity 38 seconds at 38° C. equivalent to 5.36 centistokes.

15

#### Example 2

4000 cc. of fluid was made up using 35% chemically prepared glyceryl tri-ricinoleate, 65% Cellosolve. After 6.25 gms. of KOH (0.23 oz./gal.) had been added and mixed the water tolerance was found to be 19%, a further 3.12 gms. KOH was added when the water tolerance rose to 21%. (The water tolerance of the mixture without KOH addition was 10%). The fluid thus produced had the following properties:

20 Water tolerance, 21%.

Freezing point, below -71° C.

Setting point, standard method, -66° C.

Acidity, 0.1 cc. N/10 NaOH.

25

#### Example 3

300 cc. of the glyceryl tri-ricinoleate, as prepared in Example 2, had the oil extracted by repeated washing with distilled water until no more soap could be extracted. The oil was finally dissolved in methyl ether and washed again. The ether and any water remaining in the oil was separated by distillation under reduced pressure. The product of this process was an oil somewhat lower in viscosity than the original glyceryl tri-ricinoleate. When mixed with Cellosolve in the proportion of 35% oil, 65% Cellosolve a water tolerance of 24% was obtained without the addition of any potassium hydroxide. This regained oil was again heated to 90° C. under reduced pressure and then filtered through silica gel.

40 When made up in 35% : 65% proportions a fluid having the following properties was obtained:

50 Water tolerance, 24%.

Setting point (standard test), below -66° C.

Freezing point, -73° C.

Acidity, 0.6 cc. N/10 NaOH on 20 cc. fluid.

55 The oil itself had the following characteristics:

Sap. value, 128.8.

Iodine value, 54.

60 As against the original glyceryl tri-ricinoleate which had:

Sap. value, 194.

Iodine value, 57.19.

65

#### Example 4

70 The sodium alcoholate of di-ethylene glycol mono ethyl ether was prepared by reacting 23 gms. metallic sodium with 90 gms. of the mono-ethyl-ether. The dark brown solution obtained was added to a castor oil-Cellosolve mixture in the proportions of 35% oil to 65% Cellosolve and a water tolerance of 25% was obtained immediately.

75 I claim:

1. A process for the production of a fluid for

transmission of power which comprises mixing glyceryl tri-ricinoleate and a glycol mono-ether with a substance selected from the group consisting of alkali hydroxides and alcoholates, the amount of said substance being in excess of that required to neutralise the free acidity of the tri-ricinoleate, and when neutrality is reached separating the saponification products formed by washing with water and mixing the washed oil with further glycol mono-ether.

2. A process for the production of a fluid for transmission of power from glyceryl tri-ricinoleate and the mono-ethyl-ether of diethylene glycol in the proportion of about 35% tri-ricinoleate and about 65% glycol ether, which comprises dissolving an alkali hydroxide in a small portion of the glycol ether, the amount of alkali being in slight excess of that required to neutralise the free acidity of the tri-ricinoleate, and adding the resulting solution to the tri-ricinoleate and when neutrality is reached separating the saponification products formed by washing with water and mixing the washed oil with further diethylene glycol mono-ethyl-ether to bring the proportions to 35% oil : 65% glycol ether.

3. A process for the production of a fluid for transmission of power from glyceryl tri-ricinoleate and the mono-ethyl-ether of diethylene glycol in the proportion of about 35% tri-ricinoleate and about 65% glycol ether, which comprises reacting an alkali metal with a small portion of the glycol ether, the amount of alkali being in slight excess of that required to neutralise the free acidity of the tri-ricinoleate, and adding the resulting solution to the tri-ricinoleate and when neutrality is reached separating the saponification products formed by washing with water and mixing the washed oil with further diethylene glycol mono-ethyl-ether to bring the proportions to 35% oil : 65% glycol ether.

4. A process for the production of a fluid for the transmission of power which comprises mixing together about 35% glyceryl tri-ricinoleate and about 65% diethylene glycol mono-ethyl-ether and adding an alkali metal to the mixture in excess of that required to neutralise with the alkali alcoholate formed the free acidity of the tri-ricinoleate, and when neutrality is reached separating the saponification products formed by washing with water and thereafter adjusting the

proportions of the oil and glycol ether to 35% oil and 65% glycol ether.

5. A process for the production of a fluid for transmission of power which comprises contacting glyceryl tri-ricinoleate in the presence of the mono-ethyl-ether of diethylene glycol with excess of an alkali alcoholate over that required to neutralise the free acidity of the glyceryl tri-ricinoleate, permitting the reaction to proceed until the free acid is substantially neutralised, and when neutrality is reached separating the saponification products by washing with water, and thereafter mixing the washed fluid with further glycol mono-ether.

10 6. A process for producing a power transmission fluid containing glyceryl tri-ricinoleate and mono-ethyl-ether of diethylene glycol, including the steps of mixing a small portion of the glycol employed with an excess of an alkali hydroxide over that required to neutralise the free acidity

20 of the glycol tri-ricinoleate, adding the resulting solution to the tri-ricinoleate, permitting the reaction to proceed until the free acid of the tri-ricinoleate is substantially neutralised, and when neutrality is reached separating the saponification

25 products by washing with water, and thereafter adding the remainder of said glycol to the solution.

WILLIAM PERCIVAL SMITH.

#### REFERENCES CITED

The following references are of record in the file of this patent:

#### UNITED STATES PATENTS

|    | Number    | Name           | Date          |
|----|-----------|----------------|---------------|
| 35 | 1,984,421 | Muench et al.  | Dec. 18, 1934 |
|    | 2,197,339 | Gooding et al. | Apr. 16, 1940 |
|    | 2,205,183 | Woodhouse      | June 18, 1940 |
| 40 | 2,238,045 | Fulton         | Apr. 15, 1941 |
|    | 2,249,300 | Weber          | July 22, 1941 |
|    | 2,255,208 | Fife           | Sept. 9, 1941 |
|    | 2,345,585 | Clark et al.   | Apr. 4, 1944  |
|    | 2,350,583 | Bradley        | June 6, 1944  |
| 45 | 2,386,182 | Balcar         | Oct. 9, 1945  |

#### FOREIGN PATENTS

| Number  | Country       | Date         |
|---------|---------------|--------------|
| 348,642 | Great Britain | May 11, 1931 |